

Nov. 4, 1924.

1,514,283

J. H. HASTE

FILM MAKING PROCESS

Filed April 14, 1923

FIG. 1.



FIG. 2.



INVENTOR.

James H. Haste,  
BY R. L. Stinchfield  
ATTORNEY

Patented Nov. 4, 1924.

1,514,283

# UNITED STATES PATENT OFFICE.

JAMES H. HASTE, OF ROCHESTER, NEW YORK, ASSIGNOR TO EASTMAN KODAK COMPANY, OF ROCHESTER, NEW YORK, A CORPORATION OF NEW YORK.

## FILM-MAKING PROCESS.

Application filed April 14, 1923. Serial No. 632,156.

*To all whom it may concern:*

Be it known that I, JAMES H. HASTE, a citizen of the United States of America, residing at Rochester, in the county of Monroe and State of New York, have invented certain new and useful Improvements in Film-Making Processes, of which the following is a full, clear, and exact specification.

10 This invention relates to processes of making film in which cellulosic solutions or dopes are deposited or flowed on to a film-forming face, the resulting film being stripped from such face upon evaporation of 15 the solvent. One object of the invention is to provide a relatively simple film making process in which the film-forming face is not deteriorated in spite of the fact that the chief film making material tends to cause 20 such deterioration. Other objects will hereinafter appear.

In the accompanying drawing Fig. 1 is a diagrammatic side elevation, partly in section and on a reduced scale of a typical film 25 making apparatus in which my invention may be carried out, certain parts being exaggerated in relative size for the sake of clearness.

Fig. 2 is a fragmentary sectional view of 30 a film-forming face which may be employed in my process.

Films such as those employed as supports for photographic coatings are made from cellulosic dopes,—that is, solutions of such 35 substances as cellulose nitrate, cellulose acetate or cellulose ether, these solutions containing various modifying substances.

For example, a cellulose nitrate dope may include fusel oil and a little camphor, together with such volatile solvents as methyl 40 alcohol and acetone. Examples of typical cellulose acetate and cellulose ether dopes will be found in U. S. Patents Nos. 1,342,601, Seel, June 8, 1920, and 1,217,027, Lilienfeld, 45 Feb. 20, 1917, respectively.

These dopes are customarily deposited in layers on smooth faces until enough of the volatile ingredients have evaporated to leave 50 films that can be stripped off. An endless dope-receiving face, like a drum, wheel, or belt, for example, is usually employed and travels successively past a dope-applying station and a station where the film is removed from the face, the dope setting into 55 the form of a film while traveling from the

first station to the second. In this way continuous strips of film are produced that are not limited in length by the size of the facing.

It will thus be seen that on each part of the face a section of the continuous film is formed and stripped off once during each cycle of movement of the face. The repetition of this action for a large number of times subjects the face to a severe test that tends to develop defects.

Since the film is formed in intimate contact with the face, which is as smooth and polished as possible, it reproduces the surface much as a casting reproduces a mold. 70 But if the face deteriorates so that its normally smooth surface becomes pitted or contains line depressions, then corresponding protuberances or ridges will be formed on one face of the film. Furthermore, depressions in the face may expose minute areas of metal underneath the normal face, said metal being of a nature which reacts with the dope to form compounds that enter into the film in minute quantities and impair 80 sensitive photographic coatings spread thereover.

The face most often proposed for the formation of film is highly buffed or smoothed nickel-plated copper. But it has been found that certain cellulosic dopes, like cellulose acetate, which are becoming of increasing importance, are capable under film-making conditions of deteriorating such nickel-plated copper faces. It is, therefore, highly 90 desirable to provide a process by means of which cellulose acetate films may be produced on such surfaces without deteriorating them.

I have discovered that such a process may be carried out by coating the face with a thin protecting covering before the deleterious dope is spread thereover to form the main body of the film. The protective coating unites with the main layer and forms 100 therewith the transparent sheet or film which is stripped off from the face.

By way of illustration, I shall describe one embodiment of my invention in which the protective coating is formed from a nitrocellulose dope while the main part of the film is prepared from a cellulose acetate dope, it being understood that my invention is not limited to such example, except as indicated 105 in the appended claims.

Referring to the accompanying drawing, in Fig. 1 a wheel or drum 1 is provided with a shaft 2 mounted in a bearing 21. The face of this wheel is nickel-plated copper, the outer surface of nickel being highly smoothed or buffed. In Fig. 2, 6 represents diagrammatically the layer of nickel and 7 the underlay of copper. Above the wheel 1 there is located a dope-applying station 3 comprising the usual V shaped trough, from the bottom of which the protective dope 31 is deposited in the form of an exceedingly thin film 32. This dope may conveniently be one of the usual nitrocellulose film making compositions which are well known to those skilled in the art.

As the wheel 1 is rotated in the direction of the arrow 11, the protective coating 32 is carried beneath a second dope-applying station 4 which may also comprise the usual trough from which the chief film-forming material is deposited through a slot in the bottom on to the protective coating. The conditions are such that the layer 42 formed from deleterious material 41 at station 4 is much thicker than the protective coating 32. In the preferred embodiment of my invention I use a cellulose acetate dope at station 4. The coating 32 and the layer 42 unite into one substantially integral transparent film 52 which is stripped off from the face of wheel 1 at a roll station 5.

The nickel coating 6 is satisfactorily resistant to nitrocellulose compositions and consequently remains in good condition for over very long periods as long as coating 32 is applied to it and then stripped off. Since the layer 42 of deleterious material does not directly contact with the face, it is, so to speak, insulated from it as far as harmful effects are concerned. Of course, the nitrocellulose coating, which is very thin, may contain high percentages of inflammability reducing materials, such as triphenyl phosphate, tricresyl phosphate, monochlornaphthalene, etc., as will be understood by those skilled in the art. While I have described an example of my process in connection with

a nickel-plated copper wheel, the principle thereof is applicable wherever the chief film-forming ingredients have a tendency to deteriorate the particular film-forming face which is employed, a suitable thin protective coating being first applied to the face.

Having thus described my invention, what I claim as new and desire to secure by Letters Patent is:

1. The process of producing film, made chiefly from a cellulosic dope capable under film-making conditions of deteriorating the face on which said film is formed, which comprises the steps of forming a thin protecting coating on said face from a cellulosic dope that does not deteriorate said face, forming a thicker coating from said first-named dope on said protecting coating, uniting said coatings, and finally stripping the united coatings from said face.

2. The process of producing transparent film made chiefly from a cellulose acetate dope capable under film-making conditions of deteriorating a nickel-plated copper film-forming face, which comprises the steps of first forming a thin transparent protecting coating on said face from a nitrocellulose dope that does not deteriorate said face, forming a thicker transparent coating from said cellulose acetate dope on said protecting coating, uniting said coatings to form a transparent film, and finally stripping said film from said face.

3. The process of producing film made chiefly from a cellulosic dope capable under film-making conditions of deteriorating a metallic face on which said film is formed, which comprises the steps of forming a thin protecting coating on said metallic face from a cellulosic dope that does not deteriorate said face, forming a thicker coating from said first named dope on said protecting coating, uniting said coatings, and finally stripping the united coatings from said face.

Signed at Rochester, New York this 11th day of April, 1923.

JAMES H. HASTE.